

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## MULTISTAGE PROCESS OF PULPING RAW CELLULOSIC MATERIAL

No Drawing.

Application filed February 18, 1931. Serial No. 516,843.

This invention relates to a multi-stage process of pulping raw cellulose materials, for instance, woods such as spruce and fir. Its object is the economical production of a pulp having a more desirable composition and better physical characteristics, especially tear resistance, than pulps derived from the same raw material by the usual one-step chemical pulping process, such as the sulphite, soda, or 10 kraft processes.

When solutions of sodium sulphite, especially those containing alkali, are used to liberate pulp by the cooking of raw cellulosic materials therein, it is found that the pulps derived from woods such as spruce are comparable in their composition to the usual kraft pulps. That is to say, the pulps are not very high in alpha cellulose content and are characterized by a relatively high 20 portion of pentosans.

I have found that it is highly desirable to subject the raw cellulosic material to an initial cooking or extracting operation in substantially only water before its pulping is accomplished in a sulphite cooking liquor more particularly of the non-acid variety. When the initial cooking or extracting step is carried out under the appropriate temperature conditions, I have observed that a 30 notable increase in the alpha cellulose content and a decrease in the pentosan content of the resulting pulp are effected, coupled with a marked appreciation of its tear resistance. From the standpoint of securing the best results, the initial step should be performed in water at or above its boiling point, preferably between 125° to 175° C., since lower temperatures evidently do not favor much extraction of undesirable constituents, 40 such as pentosans, from the wood, whereas higher temperatures evidently promote such extraction, but at the same time cause a transformation of the ligneous content of the wood into reaction products difficultly 45 soluble during the subsequent cook to complete fiber liberation. The transformation of the ligneous content of the wood may be caused by the organic acids generated from the pentosans, for I have noted a similar 50 transformation with acid solutions, e. g., acid

sulphite solutions, in which latter case, too, difficulty is experienced in liberating fiber from the acid-cooked wood in non-acid sodium sulphite liquors. If temperatures above 175° C. are used, it is practically impossible 55 to remove much of the lignin; but even though such higher temperatures are employed in the first step, it does not prevent the pulping action of the liquor used in the second step. The resulting pulp, however, will be brown 60 and very high in lignin. There will be no reasonable way in which the fiber can be bleached, but it could be used for purposes which do not demand a white cellulose. As an example of such a case, I can cook wood in 65 water at, say, 190° C. and remove a considerable proportion of the pentosans which are present in the original wood. The resulting mass is dark brown in color. When it is pulped with a sodium sulphite solution, I 70 have found it necessary to use a higher temperature than ordinarily employed, and that I may be compelled to go to temperatures as high as 390° or 400° F. The resulting pulp will be very low in pentosans, approximating 75 1% or less. The lignin content may range from 25% to 40%, which is considerably higher than the lignin content of most pulps, including groundwood. The lignin content of the resulting pulp, based on pulp, may even 80 be higher than that of the original wood, based on wood, because of a partial removal of material from the wood during the first and second steps in my pulping sequence. By practising the initial water cook between 85 the lower temperature limit at which little benefit accrues and the upper temperature limit at which subsequent fiber liberation is hindered, I can attain my objective, namely, an improved pulp at low cost, for the initial 90 cook or extraction requires no chemicals and the second cook may be completed in a period of time no longer than usual and with no more chemical than in a single-step cook to complete fiber liberation.

The value of my invention can at once be recognized by comparing the results obtained by cooking raw wood, such as spruce, in a straight or neutral sodium sulphite solution 95 with those realized when the raw wood under-

went an initial extraction with water, as hereinbefore described, before a cook in a neutral sodium sulphite solution under conditions similar to those maintained in the single-step 5 cooking operation. The use of a neutral sodium sulphite solution is of advantage, as it permits the two-stage cooking operation of the present invention to be carried out in a single digester, for instance, a steel digester, 10 even though a slight acidity is developed in the water used in the first step. If this acidity becomes troublesome, I can add to the water a small amount of material, such as calcium carbonate or calcium sulphite, which 15 in itself will not interfere very much with the action of the water and which will act as a buffer against the development of an undesirably high concentration of acid. In carrying out the single-step cooking operation 20 to be used as a basis of comparison, I started with spruce wood cut in the form of chips such as prepared for the customary chemical pulp-making processes. These chips were placed in a digester, covered with a 10% 25 sodium sulphite solution, and digested for six hours at a temperature of about 180° C. to produce pulp. The yield of pulp was 44% based on the weight of wood used as a raw material. The washed pulp had an alpha 30 cellulose content of 86% and a pentosan content of 7.4%. When beaten according to the procedure followed in testing kraft pulps and then formed into test sheets of waterleaf paper, the sheets were found to have an average 35 pop-strength of 213 and an average tear resistance of 139. The two-stage procedure of the present invention was initiated with spruce chips taken from the same batch as in the example run for purposes of comparison. 40 The chips were placed in a digester, drowned in water, and then cooked under confinement for four hours, at 150° C. At the end of this initial cooking operation, the chips were still hard and had practically the 45 same integrity as the raw wood. They were drained and washed free of the aqueous cooking liquor, which was brown and feculent. The washed chips were then digested in a sodium sulphite solution under conditions 50 duplicating those of the single-step comparative run. The yield of pulp was somewhat lower than the comparative run, namely, 37% based on the weight of wood used as a raw material, but the washed pulp was much superior 55 in composition, having an alpha cellulose content of 94.7% and a pentosan content of 3.6%. Test sheets made and tested in the same way as those prepared from the single-stage pulp had an average pop-strength 60 of 185 and a tear resistance of 280. An enhancement of the important physical characteristics of tear resistance thus accompanied the betterment of the composition of the pulp. 65 The slight deterioration of the strength of the pulp is of no consequence, as in actual paper

manufacture the strength of the pulp can easily be raised, if desired, by beating for a longer period of time or by properly sizing the pulp.

A pulp produced by the two-stage procedure of the present invention may be directly bleached or it may be subjected to suitable chemical refining operations prior to being bleached. The finished pulp is useful both for the preparation of high grade papers 70 and cellulose derivatives, and, as will be appreciated by those skilled in the art, commands a higher degree of utility in both these spheres of use than the usual commercial wood pulps.

The process of the present invention is not restricted to soft woods, such as spruce, fir, and poplar, but to hard woods, such as birch and maple, and to other raw cellulosic materials, such as bamboo, bagasse, or hemp. 80 In carrying out the initial cooking step, neutral materials, such as sodium nitrate, zinc chloride, sugar, etc., may be added to the water to increase the ease with which pentosan groups are removed from the wood without injury to the cellulose group. The aqueous liquor from the initial cook may be separated from the chips and the chips washed, as described in the foregoing example, but, if desired, the hot liquor associated with the 85 chips may be retained in the digester and a sufficiently concentrated solution of sodium sulphite and other desired chemicals may be added thereto to produce a secondary cooking liquor of the proper concentration. The 90 secondary cooking liquor may contain only sodium sulphite, as in the foregoing example. It may contain a subordinate proportion of alkali, such as sodium hydroxide, sodium sulphide, sodium carbonate, or even a small amount of sodium bisulphite, in which latter case the liquor will be slightly acid rather than alkaline. When the secondary chemical cooking liquor is produced in the digester from the aqueous liquor resulting from the 95 initial cook, the chemicals for such cooking liquor may be introduced into the digester by injecting or pumping them as a highly concentrated solution into the closed digester so as to conserve the heat of the digester contents. Some space may be left, as ordinarily, in the digester when it is initially charged with the raw materials, including wood and water, to accommodate the concentrated chemical solution to be added thereto, although some water extract may be discharged from the digester for such purpose after the initial cook, if the digester is initially loaded with the raw materials substantially to its 100 capacity. The chips may be partially or completely submerged in water during the initial cook. In fact, the initial cook may be conducted in an atmosphere of wet steam. In any case, volatile matters extracted from the wood may be intermittently released together 105 110 115 120 125 130

with steam from the digester and, if desired, recovered by condensation. The secondary cook should be carried out at a temperature ranging from about 150° to 200° C. and for 5 a period of from about three to ten hours, depending upon the composition and concentration of the secondary cooking liquor, the character of the raw cellulosic material used, and the modification which it has undergone 10 during the initial cook.

I claim:

1. A process which comprises cooking raw cellulosic material under superatmospheric pressure in substantially only water at a temperature above not less than 125° C., and then cooking in a solution containing sodium sulphite as the main fiber-liberating agent to complete fiber liberation.
2. A process which comprises cooking 20 wood chips under superatmospheric pressure in substantially only water at a temperature of about 125° to 175° C., and then cooking in a solution containing sodium sulphite as the main fiber-liberating agent to complete fiber 25 liberation.
3. A process which comprises cooking raw cellulosic material under superatmospheric pressure in substantially only water at a temperature not less than 125° C., and then cooking 30 in a solution containing essentially only sodium sulphite to complete fiber liberation.
4. A process which comprises steaming raw cellulosic material under superatmospheric pressure at a temperature not less than 125° 35 C., and then cooking in a substantially neutral solution of sodium sulphite to complete fiber liberation.
5. A process which comprises cooking raw 40 cellulosic material under superatmospheric pressure in substantially only water at a temperature not less than 125° C., and then cooking in a solution containing alkali and a preponderant proportion of sodium sulphite to complete fiber liberation.
- 45 6. A process which comprises cooking chipped wood under superatmospheric pressure for about four hours at about 150° C. in substantially only water, and then cooking for about six hours at about 180° C. in a 50 solution of essentially only sodium sulphite to complete fiber liberation.

In testimony whereof I have affixed my signature.

GEORGE A. RICHTER.